

1

3,246,980  
CORROSION-RESISTANT ALLOYS

Milton Stern, Indianapolis, Ind., assignor to Union Carbide Corporation, a corporation of New York  
No Drawing. Filed Mar. 23, 1964, Ser. No. 354,113  
9 Claims. (Cl. 75—134)

This is a continuation-in-part of application S.N. 225,851, filed September 24, 1962, and now abandoned, said application S.N. 225,851, being a continuation-in-part of application S.N. 821,134, filed June 18, 1959, now U.S. Patent No. 3,063,835, granted November 13, 1962, said application S.N. 821,134 being a continuation-in-part of application S.N. 732,793, filed May 5, 1958 and now abandoned.

This invention relates to corrosion-resistant alloys and particularly, to corrosion resistant alloys in which chromium is the predominant metal.

Chromium and many of its alloys, as well as titanium and many of its alloys, are noted for excellent resistance to oxidizing corrosive media. In non-oxidizing corrosive media, such as hydrochloric and sulfuric acid solutions, these metals and alloys exhibit little or no resistance. It would be most desirable to have available alloys capable of withstanding corrosive environments ranging from strongly oxidizing to weakly oxidizing or non-oxidizing. An alloy of this type would have the widest utility. For example, such an alloy would be invaluable in chemical plant equipment.

Hydrochloric and sulfuric acids are prime examples of non-oxidizing corrosive media. These acids enter into many important commercial processes. They require storing and handling equipment which combine the desirable properties cited above. If a chromium alloy, for example, were to possess resistance to non-oxidizing acid solutions, in addition to its natural endowments of lightness, strength, and resistance to oxidizing acid solutions, it would be extremely useful in such applications.

One widely used method for preventing corrosion is to add passivating inhibitors to the environment which, it is believed, operate by producing local action current to anodically polarize a metal into the passive potential region. It is not always desirable, however, to alter the composition of a solution to prevent corrosion of the equipment in which it is contained, particularly when the composition of the solution is critical or specific to some process. Such a means of preventing corrosion is limited to the particular case where the composition of the contained solution is not critical.

2

According to scientific theory, corrosion resistance can be achieved in non-oxidizing environments by artificially anodically polarizing the base metal by applying an external current (which might be termed anodic protection as opposed to cathodic protection). This method, for obvious reasons, would be extremely difficult to accomplish in chemical plant equipment.

It is, therefore, the primary object of this invention to provide alloys of chromium which are resistant to the attack of oxidizing and non-oxidizing corrosive media.

It is also an object of this invention to provide a method for increasing the resistance to non-oxidizing corrosive media of the metal chromium, and its alloys.

Other aims and advantages of this invention will be apparent from the following description and the appended claims.

In accordance with these objects a corrosion resistant alloy is provided consisting essentially of from 0.005 to 5 percent by weight in the aggregate of at least one metal selected from the group consisting of ruthenium, rhodium, palladium, osmium, iridium, platinum, rhenium, up to 10 percent molybdenum, up to 40 percent iron, up to 2 percent copper, and the balance chromium.

A preferred embodiment of the present invention is an alloy consisting essentially of 0.05 to 0.5 percent by weight in the aggregate of at least one metal selected from the group consisting of ruthenium, rhodium, palladium, osmium, iridium, platinum, rhenium, up to 10 percent molybdenum, up to 40 percent iron, up to 2 percent copper, and the balance chromium.

This alloy is characterized by excellent resistance to strong acid solutions and comparatively lower cost.

It is believed that the important factor in obtaining the desired improvement, and the principle upon which the invention operates, lies in the production of sufficient local action current to anodically polarize the alloy into the passive region. High local action currents are created by high potential differences between the electrodes of the galvanic couple and by shallow polarization curve slopes. The current required to change the potential of either cathode or anode a given amount by polarization is proportional to the cathode and anode areas which, in turn, are determined by the noble metal content of the alloy.

Table I indicates the results of noble metal additions to substantially pure chromium. Table II provides the same information as to noble metal additional to binary and tertiary chromium-base alloys. The percentages given in each case are percentages by weight of the total alloy.

TABLE I  
*Effect of noble metal additions on corrosion rate of chromium*

| Nominal Composition Percent<br>Noble Metal | Corrosion Rate (Mils/Year)             |                  |                  |                  |                  |                  |                  |                  |
|--------------------------------------------|----------------------------------------|------------------|------------------|------------------|------------------|------------------|------------------|------------------|
|                                            | Boiling H <sub>2</sub> SO <sub>4</sub> |                  |                  |                  |                  |                  | Boiling HCl      |                  |
|                                            | 5%                                     | 10%              | 20%              | 30%              | 40%              | 50%              | 60%              | 5%               |
| Cr.                                        | ( <sup>1</sup> )                       | ( <sup>1</sup> ) | ( <sup>1</sup> ) | ( <sup>1</sup> ) | ( <sup>1</sup> ) | ( <sup>1</sup> ) | ( <sup>1</sup> ) | ( <sup>1</sup> ) |
| Cr plus 0.1 Pt.                            | 1.8                                    | 1.0              | 7                | 22               | 103              | 835              | 143              | 0.7              |
| Cr plus 0.5 Pt.                            | 0.5                                    | 2.7              | 9                | 28               | 175              | 37               | —                | 0.42             |
| Cr plus 1.0 Pt.                            | —                                      | —                | 8                | —                | —                | —                | —                | 0.46             |
| Cr plus 2.0 Pt.                            | —                                      | —                | 10               | —                | —                | —                | —                | 0.42             |
| Cr plus 5.0 Pt.                            | —                                      | —                | 1.5              | —                | —                | —                | —                | 0.41             |
| Cr plus 0.5 Rh.                            | —                                      | —                | 2.8              | —                | —                | —                | —                | 0.58             |
| Cr plus 0.5 Os.                            | —                                      | —                | 64               | —                | —                | —                | —                | 16.0             |
| Cr plus 0.5 Pd.                            | —                                      | —                | 4.3              | —                | —                | —                | —                | 0.79             |
| Cr plus 0.5 Ru.                            | —                                      | —                | 5.1              | —                | —                | —                | —                | 0.84             |
| Cr plus 0.5 Ir.                            | —                                      | —                | 2.4              | —                | —                | —                | —                | 0.40             |

<sup>1</sup> Dissolved.

TABLE II  
*Effect of noble metal additions on corrosion rate of chromium-base alloys*

| Nominal Composition Percent Noble Metal   | Corrosion Rate (Mils/Year)             |                       |                        |                        |                         |                        |
|-------------------------------------------|----------------------------------------|-----------------------|------------------------|------------------------|-------------------------|------------------------|
|                                           | Boiling H <sub>2</sub> SO <sub>4</sub> |                       |                        |                        | Boiling HCl             |                        |
|                                           | 10%                                    | 20%                   | 30%                    | 40%                    | 5%                      | 10%                    |
| Cr plus 2 Cu.....                         | 2660                                   | ( <sup>1</sup> )<br>7 | ( <sup>1</sup> )<br>30 | ( <sup>1</sup> )<br>84 | ( <sup>1</sup> )<br>988 | ( <sup>1</sup> )<br>20 |
| Cr plus 2 Cu plus 0.5 Pt.....             |                                        |                       |                        |                        |                         | ( <sup>1</sup> )       |
| Cr plus 10 Mo.....                        |                                        | ( <sup>1</sup> )      |                        |                        |                         |                        |
| Cr plus 10 Mo plus 0.5 Pt.....            |                                        | 8                     | 18                     | 125                    | 0.7                     | 40                     |
| Cr plus 40 Fe plus 10 Mo.....             | 40                                     | ( <sup>1</sup> )<br>2 | 9                      | 20                     | ( <sup>1</sup> )<br>130 | ( <sup>1</sup> )       |
| Cr plus 40 Fe plus 10 Mo plus 0.5 Pt..... |                                        |                       |                        |                        |                         |                        |

<sup>1</sup> Dissolved.

In Table I, the corrosion resistance of chromium without any addition is given first to serve as a comparison. Pure chromium, it will be noted, dissolves in both boiling sulfuric acid and boiling hydrochloric acid in the concentrations indicated. It will be observed that all the noble metals tested were extremely effective in reducing the corrosion rate of chromium. The degree of effectiveness varies with the quantity of noble metal added as shown in the tables. It will be observed that as little as 0.1% by weight platinum renders chromium practically insoluble in 20% boiling sulfuric acid. As shown in Table I, the 0.5 osmium addition, while it decreases the rate drastically, is not as effective as an equal amount of platinum. It will further be observed that, in general, additions of noble metal reduce the rate of corrosion of chromium in boiling non-oxidizing acids of concentrations as high as 60%. The proportion of noble metal addition may be varied according to the anticipated use. Where contact with a more rigorous environment is anticipated, such as strong concentrations of acid, more noble metal is required. For best results in conditions where exposure to strong solutions is encountered, the additive is used in amounts of between 0.05 and 0.5%. With amounts below 0.05% noble metal addition, the desired improvement in corrosion resistance may not be sufficient to meet the particular needs. As little as 0.005% of noble metal addition may suffice for low concentration of acid, however. With amounts substantially in excess of about 5%, no marked degree of improvement results while the cost of the alloy increases considerably. The noble metals may be present either singly or in combination with each other.

In Table II, the corrosion rate of several chromium-base alloys, together with the rate of the same alloy with the platinum addition is given for comparison. It will be seen that the base alloys dissolve in moderate to strong concentration of either sulfuric or hydrochloric acid. However, with the addition of as little as 0.5% platinum to the base alloy, a very marked decrease in the rate of corrosion results. The effectiveness of the noble metal addition, as before, depends on the strength of the corrosive medium and on the amount of noble metal added. Moreover, some alloys are more effectively protected by the same amount of noble metal addition than others. An 0.5% addition of platinum, for instance, while it decreases the rate of corrosion of a chromium-base alloy containing 2 percent Cu in 40 percent boiling sulfuric acid, is not as effective as with a chromium-base alloy containing 10 percent molybdenum, or an alloy consisting of 40 percent iron, 10 percent molybdenum and the balance chromium. Additions of noble metals may also be made to chromium electrodeposit.

The alloys of the present invention may be prepared according to current metallurgical practice, although the invention is not limited by the method of preparation. The ingredients may be in any commercially pure form.

The description of the invention above has been in

terms of its specific embodiments. Modifications and equivalents will be apparent to those skilled in the art and this disclosure is intended to be illustrative of, but not necessarily to constitute a limitation upon, the scope of the invention.

What is claimed is:

1. A corrosion-resistant alloy consisting essentially of from about 0.05 to 0.5 percent by weight in the aggregate of at least one metal selected from the group consisting of ruthenium, rhodium, palladium, osmium, iridium, platinum, rhenium, up to 10 percent molybdenum, up to 40 percent iron, up to 2 percent copper, balance chromium.
2. A corrosion-resistant alloy consisting essentially of about 0.1 percent by weight platinum, and the balance chromium and incidental impurities.
3. A corrosion-resistant alloy consisting essentially of about 0.5 percent by weight platinum, and the balance chromium and incidental impurities.
4. A corrosion-resistant alloy consisting essentially of about 0.5 percent by weight palladium, and the balance chromium and incidental impurities.
5. A corrosion-resistant alloy consisting essentially of about 10 percent by weight molybdenum about 0.50 percent by weight platinum, and the balance chromium and incidental impurities.
6. A corrosion-resistant alloy consisting essentially of about 40 percent by weight iron, about 10 percent by weight molybdenum, about 0.5 percent by weight platinum, and the balance chromium and incidental impurities.
7. A corrosion-resistant alloy consisting essentially of about 2 percent by weight copper, about 0.50 percent by weight platinum, balance chromium and incidental impurities.
8. A corrosion-resistant alloy consisting essentially of about 0.1 to about 0.5 percent by weight platinum, up to 10 percent by weight molybdenum, up to 40 percent by weight iron, balance chromium and incidental impurities.
9. A corrosion-resistant alloy consisting essentially of about 0.1 to about 0.5 percent by weight platinum, about 10 percent by weight molybdenum, about 40 percent by weight iron, balance chromium and incidental impurities.

#### References Cited by the Examiner

##### UNITED STATES PATENTS

|           |         |          |       |        |
|-----------|---------|----------|-------|--------|
| 1,167,827 | 1/1916  | Kaiser   | ----- | 75—176 |
| 3,008,854 | 11/1961 | Grant    | ----- | 75—176 |
| 3,063,835 | 11/1962 | Stern    | ----- | 75—176 |
| 3,131,059 | 4/1964  | Kaarlela | ----- | 75—176 |

##### FOREIGN PATENTS

|        |        |                |
|--------|--------|----------------|
| 18,212 | 7/1914 | Great Britain. |
|--------|--------|----------------|

(Other references on following page)

**References Cited by the Applicant****UNITED STATES PATENTS**

- 2,247,755 7/1941 Hensel et al.  
2,659,669 11/1953 Muller.  
2,780,545 2/1957 Blank et al.

**OTHER REFERENCES**

ASM Metals Handbook, 1949 edition, page 22. Published by the ASM, Cleveland, Ohio.

Hansen: Constitution of Binary Alloys, McGraw-Hill Book Co., Inc., New York, 1959, pages 550, 555.  
Pietrokowsky et al., Journal of Metals, vol. 8, August 1956, pages 930-935. Published by the A.I.M.E., New York, N.Y.

**BENJAMIN HENKIN, Primary Examiner.**

**WINSTON A. DOUGLAS, Examiner.**